

Jan. 21, 1936.

J. V. STARR ET AL

**2,028,361**

## PROCESS FOR PRODUCING LUBRICATING OILS

Filed June 20, 1931



John V. Starr  
David F. Edwards

By W. E. Currie Attorney

## UNITED STATES PATENT OFFICE

2,028,361

## PROCESS FOR PRODUCING LUBRICATING OILS

John V. Starr and David F. Edwards, Elizabeth, N. J., assignors to Standard Oil Development Company, a corporation of Delaware

Application June 20, 1931, Serial No. 545,693

2 Claims. (Cl. 196—79)

This invention relates to a process for producing finished lubricating oils of high color and good cast from a lubricating oil stock treated with a selective solvent. The invention will be fully understood from the following description read in conjunction with the drawing, the sole figure of which is a diagrammatic side elevation, partly in section, showing one form of the apparatus used for carrying out the invention.

When producing lubricating oils by extraction with selective solvents such as phenol, aniline, furfural, etc., it is customary to subject the raffinate to distillation or to agitate it with a suitable washing medium in order to remove the solvent from the treated oil. The general appearance of the lubricating oil thus obtained from an originally low grade distillate is distinctly inferior and necessitates a finishing procedure of some kind.

The object of the present invention is to provide a finishing procedure whereby the solvent is separated from the raffinate and at the same time a finished lubricating oil of any desired viscosity is obtained possessing high color and excellent appearance when viewed in reflected light.

After treating mineral oil or a distillate with selective solvents the treated oil layer usually contains from 10 to 20% of the solvent depending on the solvent employed and the temperature of the treat. We have found that by mixing a small quantity, say  $\frac{1}{2}$  lb. to 1 lb. per gallon of adsorbent clay, such as fuller's earth or an acid treated or activated clay, with the treated oil, subjecting the mixture of oil and clay to distillation so as to remove the solvent with the lighter oils and subsequently separating the clay from the residual oil, not only the separation of the selective solvent from the lubricating oil is obtained, but simultaneously, a finished lubricating oil product is produced which has excellent color and cast. The distillation may be carried out either in a shell still or in a pipe still or in a combination of a shell still and a pipe still or two pipe stills, as will be understood hereinafter.

In some cases it may be desirable or economical to recover part of the solvent from the treated oil by means other than distillation, such as, for example, by washing, or it may be economical to distill off the major portion (say 90%) or even more of the solvent in a shell still then add the clay to the residual oil and submit the latter to distillation in a pipe still in the presence of clay. The preferred operation, however, is the following:

The raffinate containing some solvent is mixed

with agitation with the necessary quantity of fuller's earth or an activated clay and the slurry thus obtained is passed through heat exchangers and then through the heating coil of a pipe still where it is heated to a temperature sufficiently high to vaporize most of the solvent. The hot oil and clay mixture is then discharged into the vaporizing zone of a bubble tower held under substantially atmospheric pressure. The solvent will be taken off as an overhead product from the tower, and is condensed and returned to storage for further use. The bottoms from the atmospheric tower are further heated by passage through a separate heating coil placed in a furnace or by other suitable means to such a temperature as to vaporize the lighter portions of the oil and insure the removal of any remaining solvent. The hot bottoms containing the clay are then flashed into the vaporizing zone of a bubble tower held under high vacuum. The remaining solvent together with some light oil is obtained as overhead product from the vacuum tower, spindle oils or light motor oils are taken out as upper side stream, heavier motor oils as lower side stream and cylinder oil or heavy motor oil containing spent clay is withdrawn as bottoms, cooled and passed through a filter press to remove the clay. The procedure may be varied to produce oils of any desired viscosity. The apparatus for this preferred operation is shown in the drawing.

Referring now to the drawing, numeral 1 designates an oil storage tank, 2 a treater for treating the oil with a selective solvent, 3 the storage tank for the extract and 4 the storage tank for the treated oil. The hopper 5, mixing tank 6 and mixer 7 serve for the admixture of decolorizing clay to the treated oil. Pump 8, heat exchangers 9, 10 and tube still 11, serve for passing and heating the oil clay slurry into the vaporizing and fractionating tower 12. The overhead product (treating solvent) is removed through line 13, condensed in condenser 14 and stored in tank 15 from which it may be pumped by means of pump 16 into treater 2. The residue of distillation is removed from tower 12 through line 17 and passed by means of pump 18 through tube still 19 and line 20 provided with the pressure reduction valve 20' into the vacuum tower 21. The overhead product leaves the vacuum tower through line 22 and is condensed in condenser 23. Means such as vacuum steam jet pumps 24 or any other known means are provided for maintaining the necessary vacuum. Lines 25 and 26 serve for removing the side streams through heat exchangers 9 and 10, respectively. The residue

from the vacuum tower leaves through line 27 and is pumped by means of pump 28 through cooler 29 and filter press 30 to separate the spent clay from the treated residuum.

5 The following examples will illustrate our process:

A crude lubricating distillate from Colombia having gravity of 21.8 A. P. I., viscosity of 63 at 210° F. and viscosity index of 43 (determined by the 10 method described in the article of E. W. Dean and G. H. B. Davis, Chemical and Metallurgical Engineering, volume 36, No. 10, October 1929), was treated with 50% by volume of 100% phenol at 108° F. After agitation for about ten minutes 15 the mixture was allowed to stratify and the extract layer withdrawn. Five additional dumps of phenol each 50% by volume of the oil being treated were applied and the extract layers in each case removed as before. A raffinate yield 20 of 63.7% was obtained. A sample of the raffinate which showed 12% phenol was dephenolized by distillation, yielding dephenolized oil 56% of charge. The phenol free oil had a gravity of 25.7 viscosity of 59 seconds Saybolt at 210° F. a viscosity index of 88, but low Robinson color. The bulk of the raffinate with the 12% phenol content was placed in an agitator heated at 110-120° F. and mixed with 1/2 lb. per gallon of an activated adsorbent clay. The oil clay slurry 30 was then fed through a heating coil where the temperature was raised to 557° F. and flashed into the vaporizing chamber of a bubble tower, kept substantially under an absolute pressure of 20 mm. mercury. Substantially all of the remaining solvent was taken overhead together 35 with a relatively small amount of gas oil, a portion of the overhead being returned to the tower as reflux. The bottoms amounting to 78% of the charge were withdrawn, partially cooled (to about 40 300° F.) and the spent clay filtered therefrom. Inspection of the bottoms showed:

Gravity 26.7 A. P. I.  
Flash, °F 500° F.  
Viscosity (Saybolt) at 100° F. 760  
45 Viscosity (Saybolt) at 210° F. 74  
Viscosity index 88  
Pour, °F 25  
Color (Robinson) 6 1/2  
Color after 16 hrs. at 212° F. 6  
50 Cast Excellent

Qualitative tests in the bottoms showed no phenol present.

As a second example of carrying out our invention samples of the phenol treated Colombian oil described above were partially dephenolized by washing with NaOH solution, the major portion (about 90%) of the phenol being washed out. The residual oil amounting to about 89% of the original raffinate was blown bright at 60 150° F., mixed with clay at about 120° F., passed through the heating coil of a pipe still where it was heated to a temperature of 675° F., and flashed into the vaporizing zone of the bubble tower held at an absolute pressure of 17-18 mm. 65 of mercury, a portion of the overhead being returned to the tower as reflux.

Two similar experiments were carried out. In one case the sample of residual oil from the first still was mixed with 1/4 lb. per gallon of acid 70 treated clay and distilled in a pipe still, 83% being taken overhead and 17% obtained as bottoms. In the other case 1/4 lb. per gallon of finely powdered Attapulgus clay was added to the oil and distilled in the pipe still to obtain 80.3% 75 of overhead products and 19.7% of bottoms. The

bottoms of both experiments were cooled and filtered, yielding cylinder oils with the following inspection:

|                      | First experiment | Second experiment | 5  |
|----------------------|------------------|-------------------|----|
| Gravity              | 25.6             | 25.1              |    |
| Flash, °F            | 550              | 580               |    |
| Viscosity at 100° F. | 2802             | 2890              |    |
| Viscosity at 210° F. | 142              | 147               |    |
| Pour, °F             | 45               | 40                | 10 |
| Viscosity index      | 80               | 81                |    |
| Color (Robinson)     | 6                | 1 1/2             |    |
| Color hold           | 5 1/4            | 1 1/2             |    |
| Cast                 | Excellent.       | Excellent.        |    |

In both cases, the color stability as tested by maintaining the oil at a temperature of 212° F. for sixteen hours, was very good, and the general appearance of the oils viewed by reflected light showed a desirable olive green cast. The overhead products were rerun giving Spindle oil, light machine oil and motor oil of good quality.

In the following claims, the expression "selective solvent" is meant to designate solvents of the type of phenol, aniline, furfural, etc., which when brought in contact with the oil, selectively absorb certain undesirable constituents of unsaturated and/or aromatic character. The expression is not meant to include agents which have a chemical action on the constituents of the oil such as, for example, sulfuric acid, which not only absorbs certain constituents, but also causes polymerization and sludge formation, or other treating agents such as aluminum chloride, zinc chloride, iron chloride, and solutions thereof which cause polymerization or condensation reactions with certain constituents of the oil.

This invention is not to be limited by any theory or by the examples given by way of illustration, but only by the appended claims in which it is our intention to claim all inherent novelty of our process.

We claim:

1. Process of preparing lubricating oil from a lubricating oil stock which comprises agitating the stock with a selective solvent, separating the extract layer from the raffinate layer, subjecting the raffinate layer in the presence of the absorbed selective solvent which it contains at the time of its separation from the extract layer to fractional distillation in the presence of an adsorbent clay, and removing the adsorbent clay from the distillation residue.

2. The process of preparing lubricating oil from a lubricating oil stock which comprises treating said stock by agitation with a selective solvent, separating the extract layer from the raffinate layer, mixing said raffinate layer with an adsorbent clay in the presence of the absorbed selective solvent which it contains at the time of its separation from the extract layer to obtain a slurry, passing the slurry through an elongated narrow heating zone into an enlarged combined vaporizing and fractionating zone held under atmospheric pressure, removing substantially all of the solvent and a part of the oil as distillate, passing the residue through a second elongated narrow heating zone, discharging the heated residue into an enlarged combined vaporizing and fractionating zone held under vacuum to obtain at least one distillate and a second residue, and separating the clay from the second residue.

JOHN V. STARR.

DAVID F. EDWARDS.

75